

May 6, 1924.

1,492,804

H. P. MACDONALD ET AL

## HEAT TREATMENT OF METALS AND APPARATUS THEREFOR

Filed Dec. 23, 1916.

3 Sheets-Sheet 1



FIG. I.



FIG. 2.

**WITNESS:**

Robt. A. Litchel

INVENTOR

Harry P. Macdonald and  
Angus S. Macdonald

James A. Bradley, Lockhart & Fink,  
ATTORNEYS.

May 6, 1924.

1,492,804

H. P. MACDONALD ET AL

HEAT TREATMENT OF METALS AND APPARATUS THEREFOR

Filed Dec. 23, 1916

3 Sheets-Sheet 2



*James E. Bradley, Edward T. Tidwell*  
ATTORNEYS.

May 6, 1924.

1,492,804

H. P. MACDONALD ET AL.

## HEAT TREATMENT OF METALS AND APPARATUS THEREFOR

Filed Dec. 23, 1916

3 Sheets-Sheet 3



FIG. 4.



WITNESS:

Robt R. Kitchel



## UNITED STATES PATENT OFFICE.

HARRY P. MACDONALD, OF MONTCLAIR, NEW JERSEY, AND ANGUS S. MACDONALD, OF GREAT NECK STATION, NEW YORK, ASSIGNEES TO THE SNEAD & CO. IRON WORKS, OF JERSEY CITY, NEW JERSEY, A CORPORATION OF NEW JERSEY.

## HEAT TREATMENT OF METALS AND APPARATUS THEREFOR.

Application filed December 23, 1916. Serial No. 138,596.

*To all whom it may concern:*

Be it known that we, HARRY P. MACDONALD, of Montclair, county of Essex, and State of New Jersey, and ANGUS S. MACDONALD, of Great Neck Station, county of Nassau, and State of New York, have invented certain new and useful Improvements in the Heat Treatment of Metals and Apparatus Therefor, of which the following 10 is a specification.

This invention relates to an improvement in heat treatment of metals for tempering, bending and other operations and to apparatus for carrying out the same.

One of the primary objects of our invention is the provision of an improved practical method of determining the point of decalescence of metals undergoing heat treatment which is simple in character and 15 which can be carried out during the heat treatment of the metals by those ordinarily in charge of such operations. Stated in other words, one of the primary objects of our invention is the provision of a simple 20 practical method of determining the point of decalescence right in the machine shop or mill as a substitute for the expensive, complicated laboratory experiments which are usually undertaken by experienced 25 investigators previous to instituting any heat treatment operations in order to determine just what the heat treatment should be in the particular case.

Another object of our invention is the 30 provision of such an improved practical method by means of which the time when any metallic article reaches the point of decalescence regardless of variations in size, shape or cross-section or in chemical 35 composition, can be automatically indicated to those in charge of the heat treating operations.

Our invention also contemplates in this 40 connection, an improved apparatus of simple character which can be used in carrying out our improved method, the advantages of which will be set forth more specifically hereinafter.

In addition to the foregoing, our invention 45 is also directed to an improved method

of heat treating and bending rods or tubes, such for example as tubular front axles for automobiles and the like.

The foregoing, together with such other objects as may hereinafter appear, or are 50 incident to our invention, we obtain by means of a method and construction, the preferred embodiments of which are shown in the accompanying drawings, wherein:

Figures 1 and 2 are respectively front 55 and side elevations of rod or tube tempering apparatus such as shown and described in a co-pending application of Harry P. Macdonald and Edward Melville Huggins, Serial Number 103,627, filed June 14, 1916, 60 with our improvements shown in connection therewith; Fig. 3 is an enlarged view of details of the apparatus shown in Figure 2; Fig. 4 is a side elevation of one form of tube bending apparatus to which our invention is applied; and Figs. 5, 6 and 7 illustrate different modifications of tube bending. 65

Attention is first directed to that type of apparatus illustrated in Figures 1, 2, and 3, which is particularly adapted for the 70 tempering of rods and tubes. In brief this apparatus consists of a vertical frame-work 7 which is provided with two contact terminals A and B, suitably insulated. The upper contact A is relatively fixed while the lower contact B is movably mounted on the frame 7 by means of bolts 8 freely slidable in the slots 9, as shown in Figure 3. Each contact terminal comprises a pair of jaws 10 adapted to receive and clamp the tube or rod 11 to be heat treated, the jaws being held 75 in closed clamping position by yielding means such as springs 12. A common operating means comprising the vertical shaft 13 and hand lever 14, is provided for opening and closing the jaws, all as more fully shown and described in said copending application. 80

The positive and negative leads to the terminals are indicated at 15 and 16, current being supplied from any suitable source 85 under the control of switch mechanism 17. Intermediately of the contact terminals, the rod 11 is enclosed in a box 18, in order to prevent radiation and to maintain external 90 conditions uniform. The lower terminal B 95

is yieldingly held in raised position by such means as the counterweight 18' shown in Figure 2.

Located at the bottom of the apparatus 5 and in position to receive the heated tubes discharged therefrom is a quenching bath, such as the receptacle 19 which is filled with oil or other suitable quenching material or liquid, the receptacle being tilted so that 10 the tubes discharged therein will fall to one side by the action of gravity out of the direct path of discharge.

As thus far described, this apparatus is substantially the same as that shown and 15 described in the aforementioned application of Macdonald and Huggins, and its operation is substantially the same, to wit: the tube 11 is inserted into the jaws 10, the box 18 is closed, and then the circuit is 20 closed at switch 17, whereby the tube is heated by its internal resistance to the current of electricity flowing therethrough. When the tube has been brought to the correct temperature, the jaws are released and 25 the tube discharges into the quenching bath and is hardened.

As a general rule, metals such as steel rods, tubes and the like should be heated to what is commonly called the decalescent 30 point, which corresponds to the correct point to which it should be heated for hardening purposes. The point of decalescence of course varies with the different metals, and also with variations in chemical compositions, as for example with the carbon and 35 manganese content of steel. As previously pointed out, it is customary to conduct careful experiments to determine the decalescent points of the metal to be treated before and 40 heat treatment is attempted, and we propose to automatically determine the point of decalescence of each piece to be heat treated without the necessity of previously instituting any such experiments as are 45 customary.

In carrying out our process we take advantage of the fact that the decalescent point is somewhat analogous to the boiling point of water in that the material being 50 heated will absorb some heat thereat without its temperature being raised. In other words, the heat at the point of decalescence is that which effects the chemical and physical changes of the structure of the material and consequently it is at this point of 55 decalescence that the expansion of the material, due to the heat being supplied to it, pauses temporarily. We propose therefore to automatically indicate the instant that 60 the metal being treated reaches the point of decalescence, by indicating the point at which expansion of the metal substantially pauses. By this means we can determine both the lower and upper points of decales- 65 ence.

We accomplish this in the apparatus just described by providing an indicating mechanism C associated with the lower or movable block B. This indicating mechanism may be of any type and may set in operation any desired indicating medium, but we prefer to use a simple graduated dial 70 20 having an indicating hand 21 rotatably mounted thereon. This hand is provided with a pinion 22 which is engaged by gear 75 segment 23 rotatably mounted on the framework 7 by means of a pin 24, the end of such gear segment being in the form of a rounded shaft 25 sildably but snugly fitting into the clevis member 26 threaded into the block B. It will be seen that as the tube 11 expands under the action of the heat, the block B will be carried downward, its movement being transmitted to the hand 21. It will also be observed that the operating mechanism is so arranged as to greatly multiply the movement of the block so that the hand 21 will be caused to move quite noticeably. After turning on the electric current the operator observes the movement of 80 the hand 21 and at the instant the hand temporarily stops moving, the operator knows that the particular piece of metal being treated has reached the point of decalescence and he then cuts off the current 85 or releases the rod, either singly or together.

By such a method of automatically indicating the point of decalescence, it will at once be seen that we have obviated the necessity for conducting the slow and expensive 90 experiments heretofore noted, and have placed it within the capacity of any ordinary workman to successfully and uniformly heat treat any different kinds of metal or metals having varying chemical properties. 100 In addition to the advantages already noted, it will be apparent that the invention is particularly valuable where a large number of similar articles are to be heat treated because of the great facility with which uniform heat conditions and therefore uniform 110 product can be maintained. Thus ideal uniform heat conditions can be arrived at regardless of variations in the length, shape or section of the articles being treated, as 115 well as regardless of the particular chemical composition of the metal.

It will of course be understood by those familiar with the art that a far greater degree of accuracy can be obtained by carrying out our invention than is the case where the operator must depend upon the color of the metal in order to determine whether or not the metal has been heated to the proper degree. The value of our invention 120 is particularly increased when applied to heating processes in which the heating medium is electricity, and therefore capable of nicety in control.

It will of course be understood that our 130

invention is applicable to the heat treatment of metals for a variety of purposes. Thus for example, it is well adapted for use in bending processes such as the bending of steel tubes, in order to conveniently determine the point at which the application of further heat should be cut off and the bending instituted. Such an application of our invention can be made in connection with tube bending apparatus such as shown in Figures 4 to 7, inclusive, although it is only specifically shown in Figure 4, in which a portion of the indicating apparatus has been illustrated.

In this case the dial 20 is adjustably mounted on the rod 27 mounted adjacent to the tube to be heat treated and bent. The gear segment 23 is yieldingly held in upper position against the stop 28 by means of a spring 29 in such manner that the nose 23' of the gear segment will extend in down position so as to engage the movable contact B' mounted on the tube. As the tube 11 is heated by the current passing therethrough it expands and the upward movement of the contact B' is transmitted to the indicator hand 21 through the medium of the nose 23' in substantially the manner indicated. By adjustably mounting the dial 20 on the rod 27 it will be seen that the indicating mechanism can be readily accommodated to different spacings of contact blocks.

The remaining features of our invention have to do with the heat treatment of tubes for bending operations, and consist in heat treating the tube by its internal resistance to a current of electricity passed therethrough, while it is in position on the bending apparatus. As one means for carrying out the foregoing we have illustrated the mechanism shown in Figure 4 in which the tube 11 is supported in a fixed contact terminal or block A' so as to extend between the die or form 30 and the bending wheel 31 carried in the arm 32 pivotally mounted on the shaft 33, which in turn is supported in a suitable jaw casting or base 34. The other terminal or block B' is adjustably mounted upon the tube 11 so that it may be readily shifted so as to heat that portion of the tube only which it is necessary to heat.

After the parts have been properly positioned, the current is turned on and when the tube has been raised to the proper degree of heat, as established by the indicating mechanism, the current is turned off and the tube 11 is bent around its form or die 30, during which operation it is firmly held by the lower contact block A', while the relation between the contact B' and the indicating mechanism is such that no impediment is offered to the bending operation.

In addition to the prevention of scale and the consequent loss of material, our improved method is advantageous in that it

eliminates the complicated and expensive heating furnaces and handling mechanism usually employed in carrying out bending operations, and avoids the loss of time entailed by the use of such apparatus. Furthermore, we are enabled to carry out the bending operation at the very point when the metal has been raised to the proper degree of temperature, and we are also enabled to secure superiority and uniformity in product as will further appear.

In Figures 5 and 6, we have also shown one form of bending apparatus used for example in bending tubular front axles for automobiles, such apparatus comprising the die or form 30' and the bending rolls 31' which are adapted to be moved outwardly and downwardly. The terminal blocks A'' and B'' are adjustably mounted on the tube 11' so as to heat only the required portion of the tube and it is to be understood that indicating mechanism is arranged in cooperation with one or the other of said blocks substantially in the manner indicated in Figure 4.

In Figure 7 is illustrated still another type of apparatus which might be used to bend a tubular front axle. In this construction two fixed bottom rolls 35 are mounted in a suitable base 36 and a third roll 37 is located at a point above such rolls and mounted for vertical movement so as to bend the tube 11' in the desired manner, the stationary wing rolls 38 cooperating therewith.

It will of course be understood that in carrying out our tube bending process we fill the tube to be bent with suitable material such as sand or the like, but we prefer to use an inert material which will assist in preventing oxidation.

By our improved process of tube bending, the molecules of metal of the tube are heated uniformly throughout, thus maintaining uniform heat conditions and always insuring that every portion of the tube is in proper condition for the bending, which of course will produce not only a uniform product but also a superior product.

The term "decalescent point," as found in this specification, is employed in a broad sense and is to be understood as including what is technically more properly termed the "critical point," i. e., that temperature at which certain changes take place in the steel which place it in the proper condition for quenching in some cooling medium for hardening purposes, and at which point the steel will absorb a considerable amount of heat without corresponding rise in the temperature, and therefore, without a change in the dimensions of the steel, such for instance, as a change in the length of the piece being treated. It will be apparent that our invention will be found most useful in determining this technical "critical point,"

but since, as previously pointed out, our invention can be employed in simply determining the points of decalescence of metal, of which there are several, we have used the term "decalescent" in a broad sense.

We claim:

1. In the commercial heat treatment of metallic articles, the method of ensuring certainty of results in the condition of the metal which consists in heating the article, and in utilizing variations in the rate of physical changes of the article during heating as a medium through which the allotropic changes in the article will be indicated by the article itself.

2. In the commercial heat treatment of metallic articles, the method of ensuring certainty of results in the condition of the metal which consists in heating the article, and in utilizing variations in the rate of physical changes of the article during heating as a medium through which the allotropic changes in the article will be indicated by the article itself, and in cutting off the heat and quenching the article when the desired properties are indicated.

3. In the commercial heat treatment of metallic articles, the method of ensuring certainty of results in the condition of the metal which consists in heating the article, and in utilizing variations in the rate of physical changes of the article during heating as a medium through which the internal conditions of the article will be indicated by the article itself through indicator means associated with the article and responsive to said physical change.

4. In the commercial heat treatment of metallic articles, the method of ensuring certainty of results in the conditions of the metal which consists in suspending the article for discharge from the heating apparatus in heating the article, in indicating the internal condition of the metal by variations in the rate of physical change of the article itself through means associated with the lower end of the article and responsive to such change, and in discharging the article when the desired internal conditions are indicated.

5. In the commercial heat treatment of metallic articles, the method of ensuring certainty of results in the condition of the metal which consists in suspending the article for discharging from the heating apparatus in heating the article, in indicating the internal condition of the metal by variations in the rate of physical change of the article itself through means associated with the lower end of the article and responsive to such change, and in discharging the article when the desired internal conditions are indicated and in quenching the article.

6. In a machine for commercially heat treating metallic articles, the combination of

a releasable support for supporting the article in the machine for discharge therefrom on release, means for heating the article by its internal resistance to a passage of electric current therethrough, an indicator mechanism associated with one end of the article and adapted to translate change in dimension of the article as it is heated into an indication of temperature.

7. In a machine for commercially heat treating metallic articles, the combination of a frame, a pair of article engaging supports carried thereby, one of said supports being fixed and the other being slidable in the frame, and indicator mechanism operatively associated with an end of the article to indicate physical change in the article during heating whereby the operator may be apprised of the condition of the article by the article itself.

8. In a machine for commercially heat treating metallic articles, the combination of a frame, means for releasably supporting the article in a substantially vertical position, means for heating the article, and indicator mechanism associated with the lower end of the article and adapted to indicate physical change in the article during heating whereby the operator may be apprised of the condition of the article by the article itself.

9. In a machine for commercially heat treating metallic articles, the combination of a frame, an upper and a lower support adapted to releasably receive the article and support the same in substantially vertical position, the upper support being relatively fixed while the lower support is slidable in the frame, and indicator mechanism operated by the movement of the movable support as the latter shifts during change in physical dimension of the article whereby the operator is apprised of the temperature of the article by the article itself.

10. In the commercial heat treatment of metallic articles, the method of ensuring certainty of results in the condition of the metal which consists in heating the article and in utilizing variations in the rate of physical change of the article during heating as a medium through which the temperature of the article is indicated by the article itself, and in stopping the further heating of the article when it has reached the desired temperature.

11. The method of determining when metal, as steel or an alloy thereof, passes through a critical point, which consists in changing the heat content of the metal, determining the rate of change of dimension of the metal and noting the time of occurrence of a substantial change in the rate of change of dimension.

12. The method of determining when metal, as steel or an alloy thereof, passes

through a critical point, which consists in changing the heat content of the metal and in determining the time of occurrence of an abrupt change in the rate of change of dimension of the metal under heat.

13. The method of determining when metal, as steel or an alloy thereof, passes through a critical point, which consists in changing the heat content of the metal, not-

ing the rate of change of dimension of the metal, and noting the time of occurrence of abrupt change in said rate of change of dimension.

In testimony whereof, we have hereunto signed our names.

**HARRY P. MACDONALD.**  
**ANGUS S. MACDONALD.**